

Dec. 19, 1967

MASAO TAKAHASHI ET AL

3,359,470

METHOD OF PIEZOELECTRICALLY ACTIVATING FERROELECTRIC MATERIALS

Filed Aug. 10, 1965

2 Sheets-Sheet 1



FIG. 1

INVENTORS.  
MASAO TAKAHASHI  
FUMIO YAMAUCHI  
NORIO TSUBOUCHI  
TOMEJI OHNO

BY

Hopgood & Calmady  
ATTORNEYS.

Dec. 19, 1967

MASAO TAKAHASHI ET AL

3,359,470

METHOD OF PIEZOELECTRICALLY ACTIVATING FERROELECTRIC MATERIALS

Filed Aug. 10, 1965

2 Sheets-Sheet 2



ROOM TEMP.  
ONE MINUTE AFTER  
APPLICATION OF  
AC VOLTAGE



ROOM TEMP.  
FIVE MINUTES AFTER  
APPLICATION OF  
AC VOLTAGE



ROOM TEMP.  
TEN MINUTES AFTER  
APPLICATION OF  
AC VOLTAGE



100°C  
TEN MINUTES AFTER  
APPLICATION OF  
AC VOLTAGE

FIG.2a

FIG.2b

FIG.2c

FIG.2d

$Pb(Zr0.52 Ti0.48)O_3 + 0.1 \text{ wt. \% } Cr_2O_3$   
TIME ELAPSE AFTER THERMAL DEPOLARIZATION: ONE DAY



ROOM TEMP.  
ONE MINUTE AFTER  
APPLICATION OF  
AC VOLTAGE



ROOM TEMP.  
FIVE MINUTES AFTER  
APPLICATION OF  
AC VOLTAGE



ROOM TEMP.  
TEN MINUTES AFTER  
APPLICATION OF  
AC VOLTAGE



100°C  
TEN MINUTES AFTER  
APPLICATION OF  
AC VOLTAGE

FIG.3a

FIG.3b

FIG.3c

FIG.3d

$Pb(Zr0.52 Ti0.48)O_3 + 0.5 \text{ wt. \% } Ga_2O_3$   
TIME ELAPSE AFTER THERMAL  
DEPOLARIZATION: THREE HOURS

INVENTORS.  
MASAO TAKAHASHI  
FUMIO YAMAUCHI  
NORIO TSUBOUCHI  
TOMEJI OHNO

BY

Hopgood & Calmire  
ATTORNEYS.

3,359,470

**METHOD OF PIEZOELECTRICALLY ACTIVATING  
FERROELECTRIC MATERIALS**  
Masao Takahashi, Norio Tsubouchi, Tomeji Ohno, and  
Fumio Yamauchi, Tokyo, Japan, assignors to Nippon  
Electric Company, Limited, Tokyo, Japan, a corpora-  
tion of Japan

Filed Aug. 10, 1965, Ser. No. 478,572

 Claims priority, application Japan, Aug. 10, 1964,  
39/45,524

2 Claims. (Cl. 317—262)

## ABSTRACT OF THE DISCLOSURE

A poling process for ferroelectric materials whereby an AC electric field greater than the coercive electric field intensity and less than the breakdown field intensity of the material is applied thereto, and thereafter a DC electric field is applied, to produce improved characteristics in the material.

This invention relates to poling processes for ferroelectric materials.

The invention, with all of the objects, features and advantages thereof will be best understood by reference to the description herein set forth taken in conjunction with the accompanying drawing, in which:

FIG. 1 is a graph illustrating dependence of the electro-mechanical coupling factor in the radial mode ( $k_r$ ) on the lapse of time of a ferroelectric material whose composition can be expressed as:

$Pb(Zr_{0.52}Ti_{0.48})O_3 + 0.5$  wt. percent  $Fe_2O_3$ , and produced by the poling process when the lapse of time from the thermal depolarization process to the poling process is varied.

FIGS. 2a, 2b and 2c show hysteresis curves as viewed on a cathode-ray tube screen, of several specimens at room temperature of a ferroelectric ceramic which can be expressed as:

$Pb(Zr_{0.52}Ti_{0.48})O_3 + 0.1$  wt. percent  $Cr_2O_3$ , by subjecting the specimen to a maximum A.C. voltage of 5 kv./mm. for time intervals of 1 minute, 5 minutes, and 10 minutes, respectively, after they have been left standing in air for 24 hours at the conclusion of thermal depolarization.

FIG. 2d shows a hysteresis curve produced on a cathode-ray tube screen when a specimen having the same composition was subjected to a maximum AC voltage of 5 kv./mm. at 100° C. for 10 minutes after a time elapse of 24 hours at the conclusion of thermal depolarization.

FIGS. 3a, 3b and 3c show hysteresis curves produced on a tube screen, of several specimens at room temperature of a ferroelectric material which can be expressed as:

$Pb(Zr_{0.52}Ti_{0.48})O_3 + 0.05$  wt. percent  $Ga_2O_3$ , when the specimens were subjected to a maximum AC voltage of 5 kv./mm. for time intervals of 1 minute, 5 minutes, and 10 minutes, respectively, after being left standing in air for three hours at the conclusion of thermal depolarization, and

FIG. 3d shows such a hysteresis curve when a specimen having the same composition was subjected to a maximum A.C. voltage of 5 kv./mm. at 100° C. after a time elapse of three hours at the conclusion of thermal depolarization.

As those knowledgeable in the art are aware, ferroelectric materials in general exhibit the characteristics of both ferroelectricity and piezoelectricity. Displacement type ferroelectric materials such as are represented by barium titanate ( $BaTiO_3$ ) and lead titanate zirconate  $Pb(Zr\cdot Ti)O_3$  manifest no piezoelectricity even if a pair of electrodes are installed on the opposite surfaces of a

specimen regardless of whether they are ceramic materials produced by sintering in terms of solid phase reaction or single crystal materials produced by melting in terms of liquid phase reaction. The reason is due to the fact that the internal structure of such material is divided ferroelectrically into what may be called "ferroelectric domains."

Stated more specifically, piezoelectricity possessed by one domain has a direct bearing on the direction of the spontaneous polarization axis and the spontaneous polarization of all domains spatially distributed at random within a displacement type ferroelectric material even if a pair of electrodes are simply installed without applying a high DC electric field. Therefore, if a domain is elongated in proportion to the intensity of an externally applied electric field, another domain whose spontaneous polarization is in the opposite sense to that domain must be contracted by the same amount, with the result that no overall piezoelectricity is exhibited. In order that the piezoelectricity characteristic may be exhibited, the spontaneous polarization of these domains should be reoriented in one common direction. Furthermore, if the spontaneous polarization of all domains is reoriented in one direction, the greatest piezoelectric effect would be manifested by any given specimen.

A common means for effecting the reorientation is to apply a high intensity DC electric field to a ferroelectric material for a considerably long time interval to reorient the direction of spontaneous polarization of each domain in what is commonly called "the easy axial direction" of each domain which is the closest to the direction of the applied DC electric field. Such process is known as "poling."

All piezoelectric materials, however, do not belong to the crystallographic cubic structure, and accordingly in certain materials a stress is created during reorientation. In poling, therefore, the spontaneous polarization of each domain must be reoriented approximately in the electric field direction against this stress, with the result that it takes a long time to effect the reorientation. Consequently, two requirements must be met in order to impart the largest possible piezoelectric characteristic to a ferroelectric material, i.e., "poling" by the application of a sufficiently high intensity DC electric field, and for a long time interval.

On the other hand, it must be remembered that all ferroelectric materials have a certain electric field intensity breakdown voltage, so that "poling" for an extremely long time interval at an impressed voltage less than said breakdown voltage is required. In other words, the conventional poling process is extremely disadvantageous in that in order to increase the piezoelectric characteristic to a satisfactory degree the process is too time-consuming and strict control of the impressed voltage required for the electric field intensity near the breakdown field intensity is necessary.

In order to eliminate these disadvantages, poling at high temperatures has been the common practice. It has been the belief that increasing the temperature would make thermal agitation vigorous and would also more easily reorient the spontaneous polarization of each domain, and furthermore that the higher the temperature, the more the structure would approach the cubic structure so that reorientation would be promoted.

The present inventors have conducted many experimental tests to obtain a comparison of piezoelectricity attainable by poling at high temperatures with that at room temperature. With these experiments, the electromechanical coupling factor in the radial mode ( $k_r$ ) was adopted as a measure of the assessment of piezoelectricity as has been the common practice. Thus the larger the value of piezoelectricity, the larger became the value of  $k_r$ .

Table 1 shows the experimental result obtained in this manner.

TABLE 1

| Composition                                                                                                | Processing temperature, C. | Value of $k_r$ , percent |
|------------------------------------------------------------------------------------------------------------|----------------------------|--------------------------|
| Pb (Zr <sub>0.52</sub> Ti <sub>0.48</sub> ) O <sub>3</sub> +0.1 wt. percent Cr <sub>2</sub> O <sub>3</sub> | (*)                        | 41                       |
| Same as above                                                                                              | 100                        | 52                       |
| Pb (Zr <sub>0.52</sub> Ti <sub>0.48</sub> ) O <sub>3</sub> +0.5 wt. percent Ga <sub>2</sub> O <sub>3</sub> | (*)                        | 13                       |
| Same as above                                                                                              | 100                        | 45                       |
| Pb (Zr <sub>0.52</sub> Ti <sub>0.48</sub> ) O <sub>3</sub> +0.5 wt. percent Fe <sub>2</sub> O <sub>3</sub> | (*)                        | 33                       |
| Same as above                                                                                              | 130                        | 45                       |

\*Room temperature.

domain structure is gradually stabilized with a time elapse when the specimen is left standing in air and hence, the domain reorientation due to application of an electric field becomes more difficult to effect as time passes.

5 The present inventors investigated the manner in which the apparent spontaneous polarization (Ps. app.), the apparent residual polarization (Pr. app.), and the apparent coercive field (Ec. app.) vary with time after thermal depolarization by measuring hysteresis curves at room temperature.

10 Table 2 indicates a result of our measurement of the magnitudes of the above-mentioned characteristics appearing after a maximum AC voltage of 5 kv./mm. had been applied for one minute.

TABLE 2

| Composition                                                                                                | Elapsed time after thermal depolarization | Ps. app. ( $\mu$ C/cm. <sup>2</sup> ) | Pr. app. ( $\mu$ C/cm. <sup>2</sup> ) | Ec. app. (kv./mm.) | Remarks |
|------------------------------------------------------------------------------------------------------------|-------------------------------------------|---------------------------------------|---------------------------------------|--------------------|---------|
| Pb (Zr <sub>0.52</sub> Ti <sub>0.48</sub> ) O <sub>3</sub> +0.1 wt. percent Cr <sub>2</sub> O <sub>3</sub> | Immediately after depolarization.         | 25                                    | 21                                    | 1.5                |         |
| Same as above                                                                                              | 1 day                                     | 14                                    | 8                                     | 1.5                |         |
| Same as above                                                                                              | 14 days                                   | 12                                    | 6                                     | 0.9                |         |
| Pb (Zr <sub>0.52</sub> Ti <sub>0.48</sub> ) O <sub>3</sub> +0.5 wt. percent Ga <sub>2</sub> O <sub>3</sub> | 3 hours                                   | 13                                    | 11                                    | 1.5                |         |
| Same as above                                                                                              | 10 days                                   | 6                                     | 3                                     | 0.6                | Do.     |
| Pb (Zr <sub>0.52</sub> Ti <sub>0.48</sub> ) O <sub>3</sub> +0.5 wt. percent Fe <sub>2</sub> O <sub>3</sub> | Immediately after depolarization.         | 27                                    | 26                                    | 1.9                |         |
| Same as above                                                                                              | 1 day                                     | 18                                    | 14                                    | 1.5                |         |
| Same as above                                                                                              | 7 days                                    | 16                                    | 12                                    | 1.2                |         |
| Pb (Zr <sub>0.52</sub> Ti <sub>0.48</sub> ) O <sub>3</sub> +0.5 wt. percent Fe <sub>2</sub> O <sub>3</sub> | Immediately after depolarization.         | 24                                    | 22                                    | 2.0                |         |
| Same as above                                                                                              | 1 day                                     | 17                                    | 11                                    | 1.5                |         |

NOTE.—"Propeller" in the "remarks" column denotes a propeller type hysteresis loop depicted on the CRT screen.

The experimental results of Table 1 demonstrate that the higher the temperature in poling, the larger the value of  $k_r$  and hence, the more excellent the piezoelectrical properties become.

Since piezoelectric materials inherently have semi-conductive properties, however, poling at high temperatures is attended with some disadvantages, as follows:

(a) A decrease in the electrical resistance, causing a current to flow in the material when a voltage is applied, which may render the poling process itself impracticable, and

(b) Rigorous temperature control requirements because the piezoelectric properties change with the processing temperature.

It has been generally considered that the degree to which the spontaneous polarization of each domain is reoriented in the direction of an electric field in poling at room temperature or at high temperatures with a high intensity DC electric field applied is governed by three factors: the electric field intensity during poling, the processing time, and the processing temperature.

Another important factor besides these three factors that cannot be overlooked is the stability of the domain structure prior to poling. Stability of the domain structure of a ferroelectric material is considerably affected by the carrier after the structure has been formed. This problem is dealt with in detail in a treatise entitled "Polarization Changes During the Process of Aging in Ferroelectrics of the BaTiO<sub>3</sub> Type" by Z. Pajak and J. Stankowski, which appears in "Proceedings of the Physical Society," Dec. 1, 1958, vol. 72, Pt. 6, No. 468, pp. 1144-1146.

The research by the authors of the above treatise indicates that the hysteresis loops obtained just after thermal depolarization are much larger and rectangular in shape than those obtained after the specimen are left standing in air for many hours at the conclusion of the thermal depolarization process. This fact demonstrates that the

40 Table 2 indicates clearly the tendency of the values of Ps. app. and Pr. app. to be largest when measured immediately after thermal depolarization and to decrease gradually as the time elapse becomes longer. This experimental result demonstrates that the longer the elapse time after the thermal depolarization, the more difficult reorientation of the domain becomes.

45 Now a ferroelectric material which is heated above the Curie temperature loses its former domain structure, but a new domain structure will be formed after it is cooled and upon passing the Curie temperature. The fact that 50 the new domain structure stabilizes with elapsed time is evident from the above-mentioned reference and our experimental results shown in Table 2.

Such an increase in stability of the domain structure 55 renders reorientation due to poling difficult and thus the effect of poling is diminished. These facts are clearly indicated in our experimental results shown in FIG. 1.

FIG. 1 illustrates our experimental result with a lead titanate zirconate base ceramic material consisting of a 52 mole percent lead zirconate, 48 mole percent lead titanate, and 0.5 wt. percent Fe<sub>2</sub>O<sub>3</sub> as an additive agent and having the compositional formula:



The curve in FIG. 1 illustrates the manner in which 65 the piezoelectric characteristic expressed in the electro-mechanical coupling factor in the radial mode ( $k_r$ ) varies with the time interval between thermal depolarization and poling. Inspection of this curve readily reveals that the piezoelectric characteristic becomes reduced with an increasing time interval between thermal depolarization and poling.

70 It will be appreciated from the graph of FIG. 1 that stability of the domain structure is an important factor governing the poling effects and that if this is disregarded, 75 piezoelectric materials of the same quality could hardly

be made on a predictable basis regardless of how rigorously the electric field intensity, processing time, and processing temperature for poling are controlled. This graph further suggests that poling undertaken immediately after formation of the domain structure is extremely advantageous in that it can be effected at a relatively low electric field intensity, within a shorter time interval, and at a comparatively lower temperature.

A well known method of reorientation of the domain structure of a ferroelectric material consists of heating it above the Curie temperature to destroy the old structure and then decreasing the temperature below the Curie point thereby to form a new domain structure. This process is known as "thermal depolarization."

The manner in which the poling process effected immediately after thermal depolarization is advantageous over the conventional poling methods effected for ferroelectric materials after their domain structure has been fully stabilized will be evident from the illustration of FIG. 1.

The carrying out of the thermal depolarization process prior to the poling process however, is difficult in quantity production on an industrial scale for various reasons, among which are:

(a) Equipment for thermally depolarizing all ferroelectric materials at once and in large quantities must be installed,

(b) All ferroelectric materials must be transferred to the poling equipment as rapidly as possible after the thermal depolarization,

(c) Care must be exercised in poling so that the transfer may not be so hasty as to cause the processing temperature to vary or the internal temperature of the materials to become non-uniform and further, so that the different products are not so markedly different in dimensions as to result in significantly dissimilar cooling rates.

To conclude, prior industrial poling methods which result in the desirable features of small variations of

Further, according to the invention, a number of difficulties previously mentioned which attended the thermal depolarization process can be entirely obviated, while at the same time the advantage of poling immediately after depolarization can be completely retained.

The reasons for the improved piezoelectric properties according to this invention may be understood from the following explanation. The pre-treatment at a high intensity AC electric field causes rapid reversal of the direction of the electric field and changes the intensity of the field from time to time, and hence changes the direction of spontaneous polarization of many domains in the material. Thus, orientation of the domain structure that has been gradually stabilized with a time elapse is agitated and a newly oriented structure appears. While the direction of spontaneous polarization of each domain is varied by application of a high intensity AC electric field, stresses are created within the material, which remain for some time even after removal of the AC electric field to place the structure into an unstable condition. Since the pretreatment helps to bring about an unstable state both ferroelectrically and mechanically, succeeding application of a high intensity DC electric field facilitates reorientation of the spontaneous polarization of each domain in the direction of the electric field according to the poling process.

To demonstrate the validity of this viewpoint, the present inventors investigated the manner in which the apparent spontaneous polarization (Ps. app.), the apparent residual polarization (Pr. app.) and the apparent coercive field (Ec. app.) vary with time after application of an AC electric field regarding samples which had been left standing in air for many hours after the thermal depolarization.

Table 3 indicates our experimental results with a lead titanate zirconate ceramic which can be expressed as:

$Pb(Zr_{0.52}Ti_{0.48})O_3 + 0.5$  wt. percent  $Fe_2O_3$  when a maximum voltage of 5 kv./mm. was applied.

TABLE 3

| Elapse of time after thermal depolarization | Time interval of application of an AC electric field | Ps. app. ( $\mu C/cm^2$ ) | Pr. app. ( $\mu C/cm^2$ ) | Ec. app. (kv./mm.) |
|---------------------------------------------|------------------------------------------------------|---------------------------|---------------------------|--------------------|
| Immediately after depolarization.           | 1 minute.....                                        | 27                        | 26                        | 1.9                |
| Same as above.....                          | 5 minutes.....                                       | 28                        | 27                        | 1.9                |
| Same as above.....                          | 10 minutes.....                                      | 28                        | 27                        | 1.9                |
| 1 day.....                                  | 1 minute.....                                        | 18                        | 14                        | 1.5                |
| Same as above.....                          | 5 minutes.....                                       | 27                        | 24                        | 1.8                |
| Same as above.....                          | 10 minutes.....                                      | 29                        | 26                        | 1.9                |
| 1 week.....                                 | 1 minute.....                                        | 16                        | 12                        | 1.2                |
| Same as above.....                          | 5 minutes.....                                       | 24                        | 20                        | 1.5                |
| Same as above.....                          | 10 minutes.....                                      | 28                        | 26                        | 1.5                |

piezoelectric properties, reproducibility from product to product, and excellent piezoelectric properties of the products are attended with an impractically high number of manufacturing difficulties.

Accordingly, it is an object of this invention to provide a new depolarization method. Another object of the invention is to harness for industrial purposes the advantages of poling prior to stabilization of the domain structure.

A further object is to utilize the experimental information illustrated in FIG. 1 by providing a new depolarization method whereby easy and rapid synchronization with the poling process can be achieved.

In accordance with an aspect of the invention, the above problems are obviated by a poling process characterized in that an AC electric field in excess of the coercive electric field intensity and less than the breakdown field intensity of a ferroelectric material is applied thereto for a suitable time interval prior to poling, and thereafter a DC electric field in excess of the coercive field intensity and less than the breakdown field intensity is applied to the material.

The experimental result shown in Table 3 indicates that the values of Ps. app. and Pr. app. are decreased with increasing elapsed time after thermal depolarization and are increased with an increasing time period of application of a high intensity AC electric field to conform approximately to those of Ps. app. and Pr. app. just after the thermal depolarization if the application continues for 10 minutes.

FIGS. 2a, 2b and 2c illustrate the manner in which the hysteresis curve depicted on the cathode ray tube screen varies with time with an AC electric field applied to a sample of a lead titanate zirconate ceramic which can be expressed as:

$Pb(Zr_{0.52}Ti_{0.48})O_3 + 0.1$  wt. percent  $Cr_2O_3$  which had been left standing in air for one day after the thermal depolarization.

FIG. 2a denotes the configuration of the curve obtained when the AC electric field was applied for one minute, FIG. 2b that when it was applied for 5 minutes, and FIG. 2c that when it was applied for 10 minutes. The configuration of the curve thereafter remained substantially unchanged.

These experimental results clearly indicate the marked promotion of reorientation of the domain structure by the application of a high intensity AC electric field. The ceramic material having the compositional formula men-

obtained by varying the elapsed time after thermal depolarization, the conditions for application of a high AC electric field, and the conditions for application of a high DC electric field.

TABLE 4

| Time elapse after thermal depolarization. | Conditions for applying a high AC electric field.                         | Conditions for applying a high DC electric field                               | Electromechanical coupling factor in radial mode ( $k_r$ ), percent. |
|-------------------------------------------|---------------------------------------------------------------------------|--------------------------------------------------------------------------------|----------------------------------------------------------------------|
| Immediately after depolarization.         | Not applied.                                                              | Electric field at intensity 5.0 kv./mm. applied for 1 hr. at room temperature. | 43                                                                   |
| After one week.                           | Not applied.                                                              | Same as above.                                                                 | 33                                                                   |
| After one week.                           | Electric field at 2.0 kv./mm. applied for 5 minutes at room temperature.  | Same as above.                                                                 | 34                                                                   |
| Same as above.                            | Electric field at 2.0 kv./mm. applied for 10 minutes at room temperature. | Same as above.                                                                 | 35                                                                   |
| Same as above.                            | Electric field at 2.5 kv./mm. applied for 5 minutes at room temperature.  | Same as above.                                                                 | 35                                                                   |
| Same as above.                            | Electric field at 2.5 kv./mm. applied for 10 minutes at room temperature. | Same as above.                                                                 | 47                                                                   |
| Same as above.                            | Electric field at 3.0 kv./mm. applied for 5 minutes at room temperature.  | Same as above.                                                                 | 47                                                                   |
| Same as above.                            | Electric field at 2.5 kv./mm. applied for 10 minutes at $-78^{\circ}$ C.  | Same as above.                                                                 | 38                                                                   |
| Same as above.                            | Not applied.                                                              | Electric field at 5.0 kv./mm. applied for 1 hr. at $100^{\circ}$ C.            | 46                                                                   |

tioned immediately above was found to have an electrical resistance capable of withstanding a high intensity electric field at  $100^{\circ}$  C. FIG. 2d shows the configuration of the hysteresis curve measured at  $100^{\circ}$  C. It was proven by our experiment that changes in the configuration of the curve of FIG. 2d at  $100^{\circ}$  C. with elapsed time were less pronounced than changes in the configuration of the curve at room temperature with elapsed time and manifested appreciably larger values of Ps. app. and Pr. app. from the beginning.

The experimental result of FIG. 2d is equivalent in significance to the result shown in Table 1 which has proved that poling at high temperatures obtains more excellent piezoelectric properties than those obtained at room temperature. A comparison of FIGS. 2c and 2d further reveals that both configurations are quite similar and that the values of Ps. app. and Pr. app. are approximately of the same degree.

FIG. 3 shows similar results of our experiment as in the case of FIG. 2 with a lead titanate zirconate ferroelectric ceramic which can be expressed as:



The hysteresis curves in FIG. 3 indicate that the values of both Ps. app. and Pr. app. at room temperature increase with increased application time of an AC electric field to the ceramics and that the hysteresis curve measured with an AC voltage applied for 10 minutes at room temperature is similar in the configuration to the curve measured with the same AC voltage applied for 10 minutes at an elevated temperature.

It will be seen that these various experimental results confirm the validity of the inventors' theories. The inventors tested the effectiveness of the poling process according to this invention by cooling samples to  $-78^{\circ}$  C. The poling process at such low temperatures was also effective. In other words, the poling process according to this invention can find application for materials whose electrical resistivities are too low at room temperature, because the electrical resistivities of such materials can be sufficiently increased by cooling to a low temperature adapted for the poling. Therefore the poling process according to this invention may be said to be effective at any temperature unless the electrical resistance becomes too small to apply a high intensity electric field.

A description will now be made of an embodiment of the invention. Table 4 shows the piezoelectric properties in terms of the electromechanical coupling factor in the radial mode ( $k_r$ ) of a lead titanate zirconate ceramic consisting of a 52 mole percent lead zirconate, 48 mole percent lead titanate, and 0.5 wt. percent  $\text{Fe}_2\text{O}_3$  as an additive agent and which can be expressed as:



It will be evident from this table that (a) a large value of  $k_r$  is obtained by performing poling immediately after thermal depolarization, (b) the value of  $k_r$  is decreased with increasing time elapse after thermal depolarization, (c) the value of  $k_r$  is markedly improved by application of a high AC electric field at 2.5 kv./mm. for 10 minutes or more, and that (d) the value of  $k_r$  can also be improved by application of an AC electric field even if the temperature is lowered to  $-78^{\circ}$  C. Added for reference in the table is the result of poling by heating the material to  $100^{\circ}$  C. but the result of poling by applying a high intensity electric field is admittedly very comparable to the above-mentioned results.

While the foregoing description sets forth the principles of the invention in connection with specific apparatus, it is to be understood that the description is made only by way of example and not as a limitation of the scope of the invention as set forth in the objects thereof and in the accompanying claims.

What is claimed is:

1. A method of piezoelectrically activating a ferroelectric material characterized by comprising successive steps of applying an AC electric field of an intensity in excess of the coercive electric field intensity and less than the breakdown field intensity of said material, and applying a DC electric field of an intensity in excess of the order of the coercive electric field intensity and less than the breakdown electric field intensity of said material.
2. A poling method for piezoelectrically activating a ferroelectric material which comprises the successive steps of exposing said material to an AC electric field having an intensity in excess of the coercive electric field intensity and less than the breakdown field intensity of said material, and exposing said material to a DC electric field having an intensity in excess of the order of the coercive electric field intensity and less than the breakdown electric field intensity of said material.

#### References Cited

#### UNITED STATES PATENTS

|           |         |                |           |
|-----------|---------|----------------|-----------|
| 2,538,554 | 1/1951  | Cherry         | 317—262   |
| 2,702,427 | 2/1955  | Roberts        | 317—262 X |
| 2,706,326 | 4/1955  | Mason          | 317—262 X |
| 2,708,243 | 5/1955  | Brayer         | 310—8     |
| 3,108,211 | 10/1963 | Alleman et al. | 317—262   |

MILTON O. HIRSHFIELD, Primary Examiner.

J. A. SILVERMAN, Assistant Examiner.